

**1**

3,749,596

**METHOD FOR SEALING ANODIZED ALUMINUM**  
Chozo Yoshimura, Nara, Japan, assignor to Okuno Chemical Industry Company Limited, Higashi-ku, Osaka-shi, Japan

No Drawing. Filed May 11, 1971, Ser. No. 142,416  
Claims priority, application Japan, May 13, 1970,  
45/41,183

Int. Cl. C23f 7/06

U.S. Cl. 117—127

1 Claim 10

**ABSTRACT OF THE DISCLOSURE**

A composition for sealing aluminum oxide coating anodically formed on aluminum and aluminum base alloys comprises an aqueous solution containing at least one g./liter of oxygen acid ion of phosphorus and at least 0.2 g./liter of alkaline earth metal ion and having a pH of 2.5 to 9.0, and a method for sealing the aluminum oxide coating comprises contacting the coating with said composition at 20 to 50° C. and drying the resultant coating.

This invention relates to a composition for sealing aluminum oxide layers anodically formed on aluminum or aluminum base alloys.

The anodically formed aluminum oxide coatings are microporous and have very high adsorptive properties. Because of these characteristics, such coatings can be dyed in a wide variety of colors. However, these characteristics which facilitate coloration result in the drawback that when the colored anodized coating is put to use as it is, the coating is liable to staining and once the coating is stained, it is almost impossible to remove the stains. In order to eliminate this drawback, to improve corrosion resistance and to prevent discoloration of the colored anodized coating, it has generally been practiced to subject the anodized coating to a treatment for sealing the micropores therein.

The above-mentioned sealing treatment can be provided by treating the anodized coating with steam under an elevated pressure, with boiling water or with an aqueous solution of nickel acetate or an aqueous solution of cobalt acetate and nickel acetate at a temperature of higher than 80° C. Of these conventional methods, the treatment with high pressure steam produces a sealed coating with satisfactory properties but this involves high equipment cost and expenses. With this treatment, it is further difficult to effect continuous operation for mass production, because it is practiced on batch system, and there is another drawback that the pigment dissolves out from the colored coating. For these reasons, sealing treatment is generally carried out with boiling water or a nickel acetate bath or cobalt acetate-nickel acetate bath in recent years. However, the treatment with boiling water still permits the dye to dissolve out from the colored anodized coating, while the fact that the treatment with nickel acetate or cobalt acetate-nickel acetate bath has to be conducted at a temperature of at least 80° C. is inevitably accompanied by an increased equipment cost for heating operation when large aluminum articles are to be treated as in recent years. At any rate, all of the foregoing methods require a considerable length of time, hence inefficient.

It has also been proposed to use dichromate, molybdcic acid, water glass, metal chelate or the like, but any of these substances, unless used at a temperature of higher than 80° C., fails to achieve effective results and to reduce the treating time. The use of these substances is not of industrial advantage therefor.

Accordingly, the primary object of this invention is to provide a composition which is capable of effectively sealing an anodized coating on aluminum or aluminum

**2**

base alloys at around room temperature within a short period of time so as to impart to the coating corrosion resistance and abrasion resistance as high as heretofore been achieved.

5 The above and other objects of this invention will become apparent from the following description.

The term "anodized coating" as used herein is intended to mean an aluminum oxide coating anodically formed on aluminum or aluminum base alloys.

The sealing composition in accordance with the present invention comprises an aqueous solution containing at least one g./liter of oxygen acid ion of phosphorus and at least 0.2 g./liter of alkaline earth metal ions and having a pH of 2.5 to 9.

15 In contrast with the conventional method which requires a high temperature treatment of more than 80° C., the above-mentioned sealing composition of this invention is capable of imparting to the anodized coating higher corrosion resistance than has conventionally been provided and sufficiently high abrasion resistance when used at a treating temperature of about 20 to 50° C. for a short period of time.

The aluminum alloys used in the invention are those containing a minimum quantity of elements other than 25 aluminum. Representatives thereof are (1) Al-Cu alloys including Aluminum Association numbers 2014, 2017, 2018, 2024, 2025, 2117, 2214, etc., (2) Al-Mn alloys including Aluminum Association numbers 3003, 3002, 3105, etc., (3) Al-Si alloys including Aluminum Association numbers 4032, 4145, 4343, 4543, etc., (4) Al-Mg-Si alloys including Aluminum Association numbers 5005, 5051, 5052, 5056, 5154, 5456, 5457, 5556, 5557, 5652, 5657, etc., (5) Al-Mg-Si alloys including Aluminum Association numbers 6003, 6005, 6053, 6061, 6063, 6151, 6253, 6262, etc., (6) Al-Zn alloys including Aluminum Association numbers 7072, 7075, 7076, 7175, 7178, etc., and (7) others such as Aluminum Association numbers 8001, 8013, 8040, 8079, 8280, etc. The aluminum oxide coating anodically formed on aluminum or alloys thereof is usually 1 to 20 $\mu$  in thickness.

The sealing composition of this invention contains oxygen acid ion of phosphorus and alkaline earth metal ions. The source of the oxygen acid ion of phosphorus includes oxygen acids of phosphorus, such as hypophosphorous acid, phosphorous acid, orthophosphoric acid, pyrophosphoric acid, tripolyphosphoric acid, etc. and water-soluble salts thereof, and the alkaline earth metal ion source includes water-soluble alkaline earth metal salts. The aqueous solution of an alkaline earth metal salt of oxygen acid of phosphorus includes the both effective ions, i.e. oxygen acid ion of phosphorus and alkaline earth metal ion so that it is a preferred example of the sealing composition of this invention. Exemplary of such alkaline earth metal salts are calcium phosphate, magnesium phosphate, barium phosphate, magnesium ammonium phosphate, etc. Another example of the sealing composition of this invention is an aqueous solution containing an oxygen acid of phosphorus or water-soluble salt thereof and a water-soluble alkaline earth metal salt in combination. The water-soluble salts of oxygen acids of phosphorus other than alkaline earth metal salts includes alkali metal salts of oxygen acid of phosphorus such as sodium phosphate, potassium phosphate, sodium phosphite, sodium tripolyphosphate, sodium pyrophosphate, etc. The oxygen acids of phosphorus and water-soluble salts thereof may be used alone or in mixture. The water-soluble alkaline earth metal salt other than oxygen acid salt of phosphorus includes chlorides, carbonates, nitrates, acetates and the like of calcium, strontium, barium or magnesium. Such alkaline earth metal salts may be used alone or in combination.

It is required that the sealing composition of this invention contain at least one g./liter of oxygen acid ion of phosphorus and at least 0.2 g./liter of alkaline earth metal ions. If the amount of either one of these two kinds of ions is lower than the above, the sealing effect will not be fully achieved. As the concentration of oxygen acid ion of phosphorus increases, the sealing effect improves but if it exceeds 20 g./liter, no improvement will be achieved in sealing effect, hence uneconomical, although the use of larger amount as 50 g./liter will not be accompanied by any noticeable adverse effect. The oxygen acid ion concentration may preferably be in the range of 5 to 15 g./liter. Further the higher the concentration of alkaline earth metal ions, the greater will be the sealing effect achieved, but if it exceeds 20 g./liter, there will not be any improvement attained in the sealing effect and hence uneconomical, although no adverse effect will result. In general, the concentration of the alkaline earth metal ions may preferably be 2 to 7 g./liter.

It is required that the sealing composition of this invention have pH value of 2.5 to 9.0. If the pH of the composition is not higher than 2.5, poor sealing effect is obtained. Excess alkalinity with pH in excess of 9.0 may impart more improved corrosion resistance to the anodized coating upon sealing treatment but will cause the alkaline earth metal salt to precipitate and produce corrosion in the anodized coating. The preferred pH is in the range of 3 to 4, and the best results will be achieved with a sealing composition having a pH value in this range. The pH of the composition can be adjusted with a suitable acid or alkali, although this is dependent on what kinds of oxygen acid of phosphorus or salt thereof and alkaline earth metal salt are used. Examples of such acid or alkali used for the purpose of pH adjustment are hydrochloric acid, tartaric acid, nitric acid, sodium hydroxide, sodium carbonate, Rochelle salt, etc.

Further improvement in the corrosion resistance can be attained by addition of a specific water-soluble metal compound, water-soluble oxidizing agent or water-soluble reducing agent to the composition of this invention. The metal compound includes (1) compounds of the copper group such as  $\text{CuSO}_4$ ,  $\text{CuCl}_2$ ,  $\text{AgClO}_3$ ,  $\text{AgNO}_3$ ,  $\text{AuCl}_3$ ,  $\text{AuBr}_3$ , etc.; (2) compounds of the boron group such as  $\text{B}_2\text{O}_3$ ,  $\text{K}_2\text{B}_4\text{O}_7 \cdot 5\text{H}_2\text{O}$ ,  $\text{AlCl}_3$ ,  $\text{Al}(\text{NO}_3)_3 \cdot 9\text{H}_2\text{O}$ ,  $\text{NH}_4\text{AlCl}_4$ , etc.; (3) compounds of the titanium group such as  $\text{TiCl}_4$ ,  $\text{Ti}(\text{SO}_4)_2$ , etc.; (4) compounds of the carbon group such as  $\text{Na}_2\text{SiO}_3$ , water glass ( $\text{Na}_2\text{O} \cdot n\text{SiO}_2 \cdot n\text{H}_2\text{O}$ ),  $\text{SnCl}_2$ ,  $\text{H}_2\text{SnS}_3 \cdot 3\text{H}_2\text{O}$ ,  $\text{SnSO}_4$ ,  $\text{Pb}(\text{ClO}_3)_2$ ,  $\text{PbCrO}_4$ , etc.; (5) compounds of the nitrogen group such as  $\text{SbCl}_3$ ,  $\text{KSbO}_2$ ,  $\text{K}_3\text{SbS}_4 \cdot 9\text{H}_2\text{O}$ ,  $\text{BiNO}_3$ ,  $\text{NaBiO}_3$ , etc.; (6) compounds of the chromium group such as  $\text{CrCl}_3$ ,  $\text{CrO}_3$ , etc.



$\text{MoCl}_5$ ,  $(\text{NH}_4)_2\text{MoO}_4$ , etc.; (7) compounds of the manganese group such as  $\text{KMnO}_4$ ,  $\text{Mn}(\text{NO}_3)_2 \cdot 6\text{H}_2\text{O}$ , etc.; and (8) compounds of the iron group such as  $\text{FeCl}_3$ ,  $\text{FeSO}_4 \cdot 6\text{H}_2\text{O}$ ,  $\text{K}_3[\text{Fe}(\text{CN})_6]$ ,  $\text{CoCl}_2$ ,  $\text{Co}(\text{NO}_3)_2 \cdot 6\text{H}_2\text{O}$ ,  $\text{NiCl}_2$ ,  $\text{Ni}(\text{C}_2\text{H}_3\text{O}_2)_2 \cdot 4\text{H}_2\text{O}$ , etc. Examples of the oxidizing agent and reducing agent include cresol, formalin, hydrogen peroxide and sodium thiosulfate. Of these compounds, particularly preferable are  $\text{AlCl}_3$ ,  $\text{K}_2\text{B}_4\text{O}_7 \cdot 5\text{H}_2\text{O}$ ,  $\text{Na}_2\text{SiO}_3$ ,  $(\text{NH}_4)_2\text{MoO}_4$ ,  $\text{KMnO}_4$ ,  $\text{K}_3[\text{Fe}(\text{CN})_6]$ ,  $\text{K}_2\text{Cr}_2\text{O}_7$ , etc. These compounds are added alone or in combination to the composition of this invention in an amount of 0.1 to 8 g./liter, preferably 0.3 to 5.0 g./liter.

The present composition may be used in the same manner as with usual treatment with nickel acetate. Thus the treatment can be carried out by a simple method, for example, by immersion of an article to be treated in the present composition or by application of the composition by spraying or coating to the articles to be treated. In any case, the treatment in accordance with this invention can be conducted at a temperature of about 20 to 50° C. without requiring any high temperature, with the

resulting advantage that the operation procedure and apparatus can be substantially simplified and that large aluminum articles can be treated with great ease. Preferable temperature is in the range of 40 to 50° C. Moreover, treatment is completed within a markedly shortened time of about 5 to 15 minutes. The treatment is conducted on batch system or continuous system. For continuous operation, the sealing composition is supplied suitably so as to maintain the amounts of effective components at a constant level. Continuous operation may result in aging of the composition and variation in pH value due to reduction of acid or alkali. Acid or alkali may then be added suitably. It is also possible to use stabilizers for the respective components.

After the treatment with the present composition the article is washed with water, as required and dried.

For better understanding of the invention examples are given below, in which percentages are all by weight.

#### EXAMPLE 1

The following composition was prepared:

Sodium tripolyphosphate—5 g./l. (phosphate ion conc. 2.1 g./l.)

Calcium chloride—3 g./l. (calcium ion conc. 0.82 g./l.)

Tartaric acid—0.2 g./l.

Water—Amount necessary for making one liter solution pH—3.2

Aluminum plate of alloy prescribed in JIS-AIPI and containing more than 99.5% of aluminum, less than 0.5% of silicon and less than 0.05% of copper was anodized in 10% sulfuric acid at 20±1° C. using a current density of one A./dm.<sup>2</sup> for 50 minutes to form an anodized coating.

The plate was then immersed in the composition of Example 1 at 45° C. for 10 minutes for sealing. The sealed coating was subjected to the following tests. The results thereof are shown in Table 1 below.

##### (1) Corrosion resistance test

In accordance with JIS H 8601-1968, a test piece was placed in the device heated to 35±1° C. and 10% caustic soda was applied dropwise to the test piece. Upon lapse of a predetermined length of time, the test piece was washed with water and dried. Electroconduction was measured by a tester and the time required for removal of the coating was determined. The result was given in terms of second.

##### (2) Abrasion resistance test

In accordance with JIS H 8601-1968, the test piece was positioned at 45 degrees with a vertical direction and silicon carbide polishing agent 2C (Carborundum 2C) having a particle size of 60 to 90 mesh was dropped onto the test piece at the level of 1000 mm. from the specified funnel through a guide tube of 20 mm. in inner diameter at a constant rate of 320 g./min. Electroconductive test was performed by a tester to determine the time required for the removal of the coating. The result was expressed in terms of second.

##### (3) Spot dyeing test

Two drops of 1 g. of Anthraquinone Violet in 50 ml. of solution were applied to a test piece separately at room temperature, and the test piece was left to stand for 5 minutes and then washed with running water. The test piece was thereafter rubbed with cotton soaked with a cleansing agent for 15 seconds and then washed with water. Without subbing the test piece, it was dried with filter paper and checked for the formation of a spot. The results are represented by:

A: Spotless

B: Faint spot

C: Clear spot

## (4) Finger mark test

A solution mixture comprising 7 g. of sodium chloride, 1 g. of urea, 4 g. of 85% lactic acid, 500 cc. of methanol and 500 cc. of water was fully applied to sealed aluminum surface with a piece of gauze soaked with the solution mixture, and the liquid was wiped off the surface with dry gauze and checked for the presence of trace of the liquid. The results are represented by:

- A: Free of any trace
- B: Slight trace
- C: Fairly clear trace
- D: Very clear trace

Comparative samples prepared by the following methods were also subjected to the same tests and the results thereof are shown in Table 1.

## Comparison 1

The anodized coating the same as in Example 1 was sealed at 45° C. for 10 minutes using the following composition:

Sodium tripolyphosphate—5 g./l. (phosphate ion conc. 4.4 g./l.)

Tartaric acid—5 g./l.

Water—Amount necessary for making one liter solution pH—3.2

## Comparison 2

The anodized coating the same as in Example 1 was sealed at 45° C. for 10 minutes using the following composition:

Calcium chloride—5 g./l. (calcium ion conc. 1.8 g./l.)

Tartaric acid—0.3 g./l.

Water—Amount necessary for making one liter solution pH—3.2

## Comparison 3

The anodized coating the same as in Example 1 was sealed in boiled water maintained at 98 to 100° C. for 30 minutes.

## Comparison 4

The anodized coating the same as in Example 1 was sealed in the following composition at 90° C. for 30 minutes.

Nickle acetate—20 g./l.

$H_3BO_3$ —8.5 g./l.

Water—Amount necessary for making one liter solution pH—5.5

TABLE 1

| Sealing method | Corrosion resistance (sec.) | Abrasion resistance (sec.) | Spot dyeing | Finger mark test |
|----------------|-----------------------------|----------------------------|-------------|------------------|
| Number:        |                             |                            |             |                  |
| 1 Example 1    | 60                          | 1,200                      | B           | A                |
| 2 Comparison 1 | 20                          | 1,600                      | C           | C                |
| 3 Comparison 2 | 20                          | 1,600                      | C           | D                |
| 4 Comparison 3 | 55                          | 1,400                      | B           | A                |
| 5 Comparison 4 | 50                          | 990                        | B           | A                |
| Contrast*      | 20                          | 1,600                      | C           | D                |

\*Contrast shows the test results conducted on the anodized coating which was not sealed.

## EXAMPLE 2

The anodized coating the same as in Example 1 was sealed at 45° C. for 10 minutes using the following composition:

Sodium pyrophosphate—5 g./l. (phosphate ion conc. 2.2 g./l.)

Barium chloride—3 g./l. (barium ion conc. 1.97 g./l.)

Tartaric acid—0.2 g./l.

Water—Amount necessary for making one liter solution pH—3.2

The same tests as in Example 1 were performed on the resultant sealed coating and the results thereof are shown in Table 2, in which the results on the coating sealed by the following methods are shown for comparison.

## Comparison 5

The anodized coating the same as in Example 1 was sealed in the following composition at 45° C. for 10 minutes.

5 Sodium pyrophosphate—5 g./l. (phosphate ion conc. 2.2 g./l.)

Tartaric acid—0.2 g./l.

Water—Amount necessary for making one liter solution

10 pH—3.2

## Comparison 6

Barium chloride—3 g./l. (barium ion conc. 1.97 g./l.)

Tartaric acid—0.2 g./l.

Water—Amount necessary for making one liter solution

pH—3.2

TABLE 2

| Sealing method | Corrosion resistance (sec.) | Abrasion resistance (sec.) | Spot dyeing | Finger mark test |
|----------------|-----------------------------|----------------------------|-------------|------------------|
| Number:        |                             |                            |             |                  |
| 6 Example 1    | 60                          | 1,150                      | B           | A                |
| 7 Comparison 5 | 20                          | 1,600                      | C           | C                |
| 8 Comparison 6 | 20                          | 1,600                      | C           | D                |

## EXAMPLE 3

The anodized coating the same as in Example 1 was sealed in the following composition at 45° C. for 10 minutes:

Sodium phosphate—5 g./l. (phosphate ion conc. 1.34 g./l.)

Strontium chloride—3 g./l. (strontium ion conc. 1.65 g./l.)

35 Potassium permanganate—2 g./l.

Tartaric acid—2.6 g./l.

Water—Amount necessary for making one liter solution pH—3.2

40 The same tests as in Example 1 were performed on the resultant sealed coating and the results thereof are shown in Table 3, in which the results on the coating sealed by the following methods are shown for comparison.

## Comparison 7

The anodized coating the same as in Example 1 was sealed in the following composition at 45° C. for 10 minutes:

50 Sodium phosphate—5 g./l. (phosphate ion conc. 2.9 g./l.)

Tartaric acid—2.5 g./l.

Water—Amount necessary for making one liter solution

pH—3.2

## Comparison 8

The anodized coating the same as in Example 1 was sealed in the following composition at 45° C. for 10 minutes:

60 Strontium chloride—3 g./l. (strontium ion conc. 1.65 g./l.)

Tartaric acid—0.3 g./l.

Water—Amount necessary for making one liter solution

pH—3.2

## Comparison 9

The anodized coating the same as in Example 1 was sealed in the following composition at 45° C. for 10 minutes:

70 Potassium permanganate—5 g./l.

Tartaric acid—0.1 g./l.

Water—Amount necessary for making one liter solution

pH—3.2

TABLE 3

| Sealing method            | Corrosion resistance (sec.) | Abrasion resistance (sec.) | Spot dyeing | Finger mark test |
|---------------------------|-----------------------------|----------------------------|-------------|------------------|
| Number:                   |                             |                            |             |                  |
| 9----- Example 3-----     | 65                          | 1,200                      | B           | A                |
| 10----- Comparison 7----- | 20                          | 1,600                      | C           | C                |
| 11----- Comparison 8----- | 20                          | 1,600                      | C           | D                |
| 12----- Comparison 9----- | 20                          | 1,600                      | C           | D                |

## EXAMPLE 4

The following two types of sealing composition were prepared, in which the amount and kind of pH adjustor used were varied in accordance with the predetermined pH of the composition.

## Composition A

Disodium hydrogenphosphate—5 g./l. (phosphate ion conc. 1.33 g./l.)

Calcium chloride—3 g./l. (calcium ion conc. 1.1 g./l.)

pH adjustor—Amount necessary for the pH value shown in Table 4

Water—Amount necessary for making one liter solution

## Composition B

Sodium pyrophosphate—10 g./l. (phosphate ion conc. 4.2 g./l.)

Barium acetate—3 g./l. (barium ion conc. 1.5 g./l.)

Potassium bichromate—2 g./l.

pH adjustor—Amount necessary for the pH value shown in Table 4

Water—Amount necessary for making one liter solution

As the pH adjustor sodium hydroxide or tartaric acid was used.

The anodized coating the same as in Example 1 was sealed at 45° C. for 10 minutes using the above compositions having pH values changed and the tests were conducted in the same manner as in Example 1 with the results shown in Table 4 below.

TABLE 4

| Composition    | pH | Corrosion resistance (sec.) | Abrasion resistance (sec.) | Spot dyeing | Finger mark test |
|----------------|----|-----------------------------|----------------------------|-------------|------------------|
| Number:        |    |                             |                            |             |                  |
| 13----- A----- | 3  | 60                          | 1,200                      | B           | A                |
| 14----- B----- | 3  | 60                          | 1,150                      | B           | A                |
| 15----- A----- | 4  | 60                          | 1,200                      | B           | A                |
| 16----- B----- | 4  | 70                          | 1,150                      | B           | A                |
| 17----- A----- | 6  | 40                          | 1,050                      | B           | A                |
| 18----- B----- | 6  | 45                          | 1,150                      | B           | A                |
| 19----- A----- | 8  | 80                          | 950                        | B           | B                |
| 20----- B----- | 8  | 85                          | 1,020                      | B           | B                |
| 21----- A----- | 10 | 90                          | 850                        | C           | D                |
| 22----- B----- | 10 | 90                          | 900                        | C           | C                |

## EXAMPLES 5 TO 24

The following sealing compositions were prepared.

## Composition of Example 5

Phosphorous acid—3 g./l. (phosphate ion conc. 2.9 g./l.)

Calcium chloride—2 g./l. (calcium ion conc. 0.73 g./l.)

Rochelle salt—8 g./l.

Water—Amount necessary for making one liter solution pH—3.2

## Composition of Example 6

Sodium phosphite—5 g./l. (phosphate ion conc. 1.82 g./l.)

Strontium chloride—3 g./l. (strontium ion conc. 0.98 g./l.)

62% HNO<sub>3</sub>—7.6 g./l.

Water—Amount necessary for making one liter solution pH—3.0

## Composition of Example 7

Calcium hypophosphite—10 g./l. (phosphate ion conc. 6.2 g./l. Calcium ion conc. 3.8 g./l.)

Calcium nitrate—5 g./l. (calcium ion conc. 2.62 g./l.)

Rochelle salt—5 g./l.

Water—Amount necessary for making one liter solution pH—3.1

## Composition of Example 8

Potassium hypophosphite—15 g./l. (hypophosphite ion conc. 6.8 g./l.)

Magnesium nitrate—10 g./l. (magnesium ion conc. 2.8 g./l.)

36% HCl—1.2 g./l.

Water—Amount necessary for making one liter solution pH—3.1

## Composition of Example 9

Sodium pyrophosphate—20 g./l. (pyrophosphate ion conc. 7.8 g./l.)

Barium acetate—20 g./l. (barium ion conc. 8.7 g./l.)

36% HCl—9 g./l.

Water—Amount necessary for making one liter solution pH—3.2

## Composition of Example 10

20 Phosphoric acid—30 g./l. (phosphate ion conc. 28.9 g./l.)

Calcium acetate—30 g./l. (Calcium ion conc. 8.2 g./l.)

Rochelle salt—100 g./l.

Water—Amount necessary for making one liter solution pH—3.1

## Composition of Example 11

Barium phosphate—40 g./l. (phosphate ion conc. 12.6 g./l. Barium ion conc. 27.4 g./l.)

Strontium carbonate—4 g./l. (strontium conc. 1.62 g./l.)

Conc. HCl—4 g./l.

30 Water—Amount necessary for making one liter solution pH—3.2

## Composition of Example 12

35 Calcium hydrogenphosphate—50 g./l. (phosphate ion conc. 27.6 g./l. Calcium ion conc. 11.62 g./l.)

Barium carbonate—5 g./l. (barium ion conc. 1.52 g./l.)

98% H<sub>2</sub>SO<sub>4</sub>—11.7 g./l.

Water—Amount necessary for making one liter solution pH—3.0

## Composition of Example 13

40 Sodium phosphate—3 g./l. (phosphate ion conc. 1.74 g./l.)

Magnesium chloride—30 g./l. (magnesium ion conc. 7.66 g./l.)

Tartaric acid—0.2 g./l.

Water—Amount necessary for making one liter solution pH—3.3

## Composition of Example 14

50 Sodium tripolyphosphate—30 g./l. (phosphate ion conc. 12.5 g./l.)

Strontium chloride—5 g./l. (strontium ion conc. 1.63 g./l.)

62% HNO<sub>3</sub>—6.2 g./l.

Water—Amount necessary for making one liter solution pH—3.2

## Composition of Example 15

60 Phosphorous acid—50 g./l. (phosphate ion conc. 48.3 g./l.)

Calcium chloride—3 g./l. (calcium ion conc. 1.09 g./l.)

Cupric sulfate—30 g./l.

Sodium hydroxide—21.5 g./l.

Water—Amount necessary for making one liter solution pH—3.2

## Composition of Example 16

Sodium phosphite—40 g./l. (phosphate ion conc. 14.56 g./l.)

70 Strontium chloride—5 g./l. (strontium ion conc. 1.63 g./l.)

Titan trichloride—40 g./l.

Sodium carbonate—40 g./l.

Water—Amount necessary for making one liter solution pH—3.3

75 pH—3.3

## Composition of Example 17

Calcium hypophosphite—30 g./l. (hypophosphite ion conc. 22.2 g./l. Calcium ion conc. 7 g./l.)  
 Calcium nitrate—10 g./l. (calcium ion conc. 5.25 g./l.)  
 Stannous chloride—50 g./l.  
 Sodium carbonate—2 g./l.  
 Water—Amount necessary for making one liter solution pH—3.0

## Composition of Example 18

Potassium hypophosphite—20 g./l. (hypophosphite ion conc. 12.1 g./l.)  
 Magnesium nitrate—20 g./l. (magnesium ion conc. 9.67 g./l.)  
 Ammonium vanadate—3 g./l.  
 Rochelle salt—1.1 g./l.  
 Water—Amount necessary for making one liter solution pH—3.2

## Composition of Example 19

Sodium pyrophosphate—10 g./l. (pyrophosphate ion conc. 7.7 g./l.)  
 Barium acetate—30 g./l. (barium ion conc. 13.1 g./l.)  
 Antimony trichloride—5 g./l.  
 NaOH—0.5 g./l.  
 Water—Amount necessary for making one liter solution pH—3.2

## Composition of Example 20

Phosphoric acid—5 g./l. (phosphate ion conc. 4.8 g./l.)  
 Calcium acetate—40 g./l. (calcium ion conc. 17.4 g./l.)  
 Potassium dichromate—10 g./l.  
 Rochelle salt—20 g./l.  
 Water—Amount necessary for making one liter solution pH—3.0

## Composition of Example 21

Barium phosphate—3 g./l. (phosphate ion conc. 0.95 g./l., barium ion conc. 2.05 g./l.)  
 Strontium carbonate—50 g./l. (strontium ion conc. 2 g./l.)  
 Antimony molybdate—20 g./l.  
 36% HCl—48 g./l.  
 Water—Amount necessary for making one liter solution pH—3.1

## Composition of Example 22

Calcium hydrogenphosphate—50 g./l. (phosphate ion conc. 19.2 g./l. calcium ion conc. 7.93 g./l.)  
 Barium carbonate—3 g./l. (barium ion conc. 0.91 g./l.)  
 Potassium permanganate—3 g./l.  
 98% H<sub>2</sub>SO<sub>4</sub>—7.3 g./l.

Water—Amount necessary for making one liter solution pH—3.2

## Composition of Example 23

Sodium phosphate—3 g./l. (phosphate ion conc. 1.74 g./l.)  
 Magnesium chloride—50 g./l. (magnesium ion conc. 12.7 g./l.)  
 Iron alum—3 g./l.  
 Rochelle salt—16 g./l.

Water—Amount necessary for making one liter solution pH—3.1

## Composition of Example 24

Sodium tripolyphosphate—3 g./l. (phosphate ion conc. 1.25 g./l.)  
 Strontium chloride—3 g./l. (strontium ion conc. 0.974 g./l.)  
 Formalin—50 g./l.  
 62% HNO<sub>3</sub>—4.8 g./l.  
 Water—Amount necessary for making one liter solution pH—3.2

The anodized coating the same as in Example 1 was sealed at 45° C. for 10 minutes using the above compositions of Examples 5 to 24 and the same tests as in Example 1 were performed in the same manner as in Example 1 with the results shown in Table 5 below.

TABLE 5

|    | Composition | Corrosion resistance (sec.) | Abrasion resistance (sec.) | Spot dyeing | Finger mark test |
|----|-------------|-----------------------------|----------------------------|-------------|------------------|
| 10 | Number:     |                             |                            |             |                  |
| 22 | Example 5   | 60                          | 1,100                      | B           | A                |
| 24 | Example 6   | 55                          | 1,250                      | B           | A                |
| 25 | Example 7   | 55                          | 1,100                      | B           | A                |
| 26 | Example 8   | 60                          | 1,100                      | B           | A                |
| 27 | Example 9   | 60                          | 1,150                      | B           | A                |
| 28 | Example 10  | 60                          | 1,150                      | B           | A                |
| 29 | Example 11  | 60                          | 1,150                      | B           | A                |
| 30 | Example 12  | 60                          | 1,200                      | B           | A                |
| 31 | Example 13  | 60                          | 1,100                      | B           | A                |
| 32 | Example 14  | 60                          | 1,050                      | B           | A                |
| 33 | Example 15  | 65                          | 1,200                      | B           | A                |
| 34 | Example 16  | 65                          | 1,200                      | B           | A                |
| 35 | Example 17  | 70                          | 1,200                      | B           | A                |
| 36 | Example 18  | 65                          | 1,150                      | B           | A                |
| 37 | Example 19  | 70                          | 1,200                      | B           | A                |
| 38 | Example 20  | 70                          | 1,150                      | B           | A                |
| 39 | Example 21  | 70                          | 1,200                      | B           | A                |
| 40 | Example 22  | 65                          | 1,200                      | B           | A                |
| 41 | Example 23  | 70                          | 1,150                      | B           | A                |
| 42 | Example 24  | 70                          | 1,200                      | B           | A                |

## EXAMPLE 25

The following composition was prepared:

Sodium phosphite—10 g./l. (phosphite ion conc. 3.65 g./l.)  
 Magnesium chloride—3 g./l. (magnesium ion conc. 0.35 g./l.)  
 Tartaric acid—5 g./l.  
 Water—Amount necessary for making one liter solution pH—3.5

The anodized coating the same as in Example 1 was sealed at temperature shown in Table 6 below for 10 minutes using the above composition and the tests performed in the same manner as in Example 1 gave the following results.

TABLE 6

|    | Temperature (° C.) | Corrosion resistance (sec.) | Abrasion resistance (sec.) | Spot dyeing | Finger mark test |
|----|--------------------|-----------------------------|----------------------------|-------------|------------------|
| 45 | Number:            |                             |                            |             |                  |
| 43 | 20                 | 50                          | 1,150                      | B           | A                |
| 44 | 30                 | 55                          | 1,100                      | B           | A                |
| 45 | 40                 | 60                          | 1,150                      | B           | A                |
| 46 | 50                 | 60                          | 1,200                      | B           | A                |
| 47 | 60                 | 60                          | 1,200                      | B           | A                |
| 48 | 70                 | 60                          | 1,200                      | B           | A                |

What is claimed is:

1. A method for sealing aluminum oxide coating anodically formed on aluminum and aluminum base alloy, which comprises contacting said coating with a composition consisting essentially of an aqueous solution containing at least one g./liter of oxygen acid ion of phosphorus and at least 0.2 g./liter of alkaline earth metal ion and having a pH of 2.5 to 9.0 at 20 to 50° C., and drying the resultant coating.

## References Cited

## UNITED STATES PATENTS

2,528,787 11/1950 Roland \_\_\_\_\_ 148—6.15 R  
 3,015,593 1/1962 Jayne \_\_\_\_\_ 148—6.15 R

65 RALPH S. KENDALL, Primary Examiner

U.S. Cl. X.R.

204—35 N; 148—6.27